

Sept. 13, 1938.

W. A. JENNINGS

2,129,769

METHOD OF CONSTRUCTING UPRIGHT CONCRETE WALLS

Filed July 27, 1936



Inventor

William A. Jennings  
by Oliver & Hague Atty's.

## UNITED STATES PATENT OFFICE

2,129,769

## METHOD OF CONSTRUCTING UPRIGHT CONCRETE WALLS

William Allen Jennings, Des Moines, Iowa, assignor to Economy Forms Corporation, Des Moines, Iowa, a corporation of Iowa

Application July 27, 1936, Serial No. 92,755

4 Claims. (Cl. 25—154)

The object of my invention is to provide an improved method of constructing upright concrete walls having a relatively great degree of strength and durability and at relatively low cost for material and workmanship.

More specifically, it is my object to provide a method of this character in which the exposed surface of the finished wall will be relatively moisture resisting and of finished and ornamental appearance and free from bubble holes or other depressions which are usually present in such walls, and which exposed surface may, if desired, be ornamented in various colors or patterns.

15 My invention consists in the construction, arrangement and combination of the various parts of the device, whereby the objects contemplated are attained, as hereinafter more fully set forth, pointed out in my claims, and illustrated in the 20 accompanying drawing, in which:

Figure 1 shows a vertical transverse sectional view through two mold forms supported in spaced apart position and having the material for forming a supporting concrete wall between said mold forms;

25 Figure 2 shows a similar view of one of the mold forms moved to spaced apart position relative to the supporting wall;

Figure 3 shows a similar view with the concrete 30 material for forming a supplemental wall poured into the space between the supporting wall and the said mold form;

Figure 4 shows a vertical transverse sectional view through a section of the supporting wall and the supplemental wall, and illustrating the tie wires for supporting the supplemental wall when in easily broken condition in upright position against the supporting wall; and

Figure 5 shows a similar view of the completed 40 wall with the cement coating applied to the exposed surface of the supplemental wall.

Referring to the accompanying drawing, I have used the reference numeral 10 to indicate generally a sheet metal mold form of the kind now 45 in common use and which is customarily employed for forming upright walls and other concrete structures. These mold forms are usually provided with outwardly extended flanges formed 50 with perforations 11, and they are usually supported by structural beams, such, for instance, as shown at 12, and the forms are supported on these structural beams by clamping devices indicated generally by the reference numeral 13 55 which connect the structural members 12 with

the mold forms 10 and thereby support the mold forms in an upright position.

In connection with the use of these mold forms it is also customary to provide spacing bars. The spacing bar is indicated generally by the reference numeral 14 and is provided with openings through which locking pins 15 are extended. These pins go through the openings 11 in a mold form, and also through the openings 16 in the spacing bars, and these spacing bars perform the 10 function of holding the mold forms in properly spaced apart position.

Mold forms of this general character are in common use, and one example may be found in my co-pending application No. 673,214 filed May 27, 1933.

In practice with my improved method I first erect two mold forms in spaced apart position and hold them in said position by the structural members on the outer faces thereof and by the 20 spacing rods extended through them. For the purpose of practicing my improved method I also place within the space between the mold forms a series of tie wires 17 which are supported at one end by one of the mold forms, and the other 25 end is bent for a considerable distance in position parallel with and against the adjacent inner surface of the other mold form. I then pour concrete of the usual kind into the space between the mold forms and permit same to set and harden, thereby forming what I have herein referred to as the supporting wall. After this supporting wall has properly set and hardened (in practice I usually let it set and harden for three or four days) I then remove the outer mold form 30 and straighten out the tie wires to the position indicated in Figure 2. I then replace the said mold form to a position slightly spaced apart from the supporting wall, as indicated in Figure 2. In this position it may be supported wholly by 40 the spacing bars 14 and pins 15, although, if desired, it may be supported also by the structural members and fastening devices 12 and 13.

When the supporting wall and mold forms are in the position shown in Figure 2, I then fill the 45 space with concrete in the usual manner, and when this has been done it will be noted that the tie wires are firmly imbedded in both the supporting wall and in what I have termed the supplemental wall on the outer face of the supporting wall. When the supplemental wall is in a fragile, easily broken or crumbled condition and/or before the supplemental wall has fully set, I remove the adjacent mold form. When thus removed the supplemental wall is in such 50 55

condition that the tie wires will support it in its upright position and, yet, it is wet, somewhat fragile and is being subjected to the chemical action which causes it to firmly set.

5 While the supplemental wall is in said condition I apply a coating of neat cement and water to the exposed surface thereof. In applying this coating I preferably employ pressure. In many instances I have taken the neat cement and water 10 in what might be termed plastic condition, and by hand rubbed and pressed it against the supplemental wall. This, however, may be done with trowels or other implements.

Immediately after applying this neat cement 15 coating 18 there occurs a chemical reaction and a physical bonding between the coating and the supplemental wall when both are in the condition described.

The essential constituents of "Portland" cement are three in number; lime, silica, and alumina. These compounds combine during the 20 manufacturing process to form tricalcic aluminate, tricalcic silicate, and dicalcic silicate. All of these compounds are unstable and upon being 25 wetted they rearrange at different speeds.

Tricalcic silicate reacts first with the water, forming gelatinous calcium hydrate and gelatinous silica. This reaction constitutes the initial 30 set of the cement, taking place in about three hours' time. As the hydration (combination with water) continues, the gelatinous materials form a strong bond between the particles of sand and crushed rock. The tricalcic aluminate reacts at the same speed as the tricalcic silicate but does 35 not produce a strong bond. The dicalcic silicate acts only after several months' time, therefore, all cement gets stronger as time passes.

The neat cement plastic coating will adhere perfectly to the fresh, barely set supplemental 40 wall while it is in its said condition, because the gelatinous substances of the neat cement and the wall will intermingle and, upon hardening, form a tough and perfect bond exactly similar to the bond between said particles of the wall itself. 45 This type of attraction is infinitely stronger and better than any possible sort of physical bond.

During the application of the neat cement coating to the wall I preferably apply pressure for the purpose of forcing the coating into air 50 holes, pits or cracks in the exposed surface of the supplemental wall, thereby applying in addition to the chemical bonding, a physical bond due to the clinching of the coating into said air holes, etc.

The application of the neat cement coating 55 before described produces another advantageous result, in that it makes the exposed surface more moisture resistant because said air holes, etc., have become filled with neat cement which presents a more moisture resistant surface than that of the concrete wall.

In practice I have found that with this method a wall of this character may be constructed of highly ornamental character, and this is done by using ordinary dyes or coloring matter in the 60 neat cement coating, thereby giving to the exposed surface of the wall any desired color. Furthermore, while this cement coating is in its plastic condition during or after its application 65 to the supplemental wall, various patterns may be formed in it, and it may be rough and irregular in outline simulating various classes of natural stone.

In practice with my improved method I have 70 demonstrated that an upright wall constructed in

accordance with my improved method is relatively strong and durable. More particularly, I have demonstrated that it can be constructed at a minimum of cost because the outer mold form 5 may be replaced by simply hanging it upon the spacing bars supported in the set and hardened supporting wall, and the amount of labor and expense required in applying the coating of plastic neat cement to the surface is not appreciably greater than that which would be required in 10 filling up the holes in said surface left upon removal of the spacing bars.

I have found in actual practice that the proper time for the removal of the mold form from the exposed surface of the supplemental wall may 15 be determined in a practical way by permitting the supplemental wall to commence its process of setting and hardening for a period of about three hours. I then move a portion of the mold form away from the supplemental wall. If the 20 cement sticks to the surface of the metal form, then I immediately replace the metal form. This operation is repeated after fifteen or twenty minutes, and when the mold form can be removed without having the concrete adhere to it, 25 the proper time has arrived for removing the metal form bodily and at once applying the neat cement coating.

Almost immediately after the concrete is 30 poured and permitted to come to rest, the chemical action of setting and hardening commences. At the early stages of this initial setting there is formed between the grains of sand a gelatinous substance. At first this gelatinous substance is in such condition that it has almost no binding 35 effect. It, however, continues to become thicker and harder, and after about three hours it has become thick and hard enough to give to the concrete what is commonly known as the initial set, and when this initial set takes place, the mass 40 of cement is in condition where it may be easily crumbled or broken off. At this stage in the setting and hardening of the cement and upright wall, unsupported, would crumble and fall. It is, however, at this stage of the setting and hardening process that the neat cement coating must 45 be applied in order to produce the desired result.

When the supplemental wall is in said condition I apply the coating containing neat cement and water in the proportions of about one part of 50 cement and one part of water, and when this is pressed against the exposed surface of the supplemental wall, it then commences its process of setting and the formation of gelatinous substances. Thereupon the gelatinous substances contained 55 in the coating and which are just commencing their process of setting and hardening, produce the result that the comparatively soft and fluid gelatinous substances of the coating will chemically combine with the comparatively thicker 60 and stiffer gelatinous substances of the supplemental wall and thereby cause the coating to become an integral part of the supplemental wall. I have demonstrated that if the setting and hardening act of the gelatinous substances of the supplemental wall is permitted to continue for a period of five or six hours, or until the gelatinous substances in the supplemental wall have become sufficiently set so that the gelatinous substances of the coating will not penetrate and 65 chemically unite with it, then the coating will adhere to the supplemental wall only by physical entanglement or clinching and may be easily broken away or removed from the supplemental wall.

By the term "neat cement" as herein employed I mean any mixture of cement and water, including such additions thereto as may be desirable, such, for instance, as color or other ingredients which will not alter the chemical reactions which necessarily take place in the practice of my improved method.

I claim as my invention:

1. The method of constructing an upright concrete wall, which consists in erecting two mold forms spaced apart, extending spacing bars through the mold forms, placing tie wires between the mold forms, pouring Portland cement concrete between the forms for forming an upright supporting concrete wall, permitting it to set and harden, moving one of the mold forms outwardly from the supporting wall, bending the tie wires out into the space between the wall and mold form, then pouring Portland cement concrete into the space between the supporting wall and the latter mold form, then removing the latter mold form while the cement is in easily broken or crumbled condition and its gelatinous substances have not fully hardened, the supplemental wall being supported in its upright position by said tie wires and spacing bars, removing any portion of the spacing bars that may project a substantial distance beyond the exposed surface of the supplemental wall and then applying a coating of Portland cement in plastic condition to said exposed surface while said wall is in said condition, to thereby form a chemical and physical bond or union between said wall and coating.
2. The method of constructing upright concrete walls, which consists in providing mold forms spaced apart, in upright position, placing tie devices in said space, pouring Portland cement concrete between the mold forms and permitting it to set and harden, then moving one of the mold forms to position spaced apart from the concrete and supporting it in said position and causing said tie devices to extend across the space between the concrete and the said form that has been moved, then pouring Portland cement concrete into said space and permitting the concrete to remain in said space until the gelatinous substances formed therein have become sufficiently hardened to serve as a binder to hold the particles of the concrete together in a mass which is easily broken or crumbled and which would not support its own weight in the form of an upright wall of substantial height but which will be thus supported by the previously formed concrete wall and the tie devices, then removing one of the mold forms and supporting the concrete in upright position from the side of the concrete opposite from the exposed surface, then applying to said exposed surface a coating of Portland cement in thin plastic condition and thereby causing the gelatinous substances in the coating in their initial process of formation, to chemically combine with the partially hardened gelatinous substances of the concrete.

3. The method of constructing upright concrete walls, which consists in providing mold forms spaced apart, in upright position, placing supporting devices in said space, pouring Portland cement concrete between the mold forms and permitting it to set and harden, then moving one of the mold forms to position spaced apart from the concrete and supporting it in said position and causing said supporting devices to extend across the space between the concrete and the said form that has been moved, then pouring Portland cement concrete into said space and permitting the concrete to remain in said position until the gelatinous substances formed therein have become sufficiently hardened to serve as a binder to hold the particles of the concrete together in a mass which is easily broken or crumbled, but which will be thus supported by the previously formed concrete wall and the supporting devices, then removing one of the mold forms and supporting the concrete in upright position from the side of the concrete opposite from the exposed surface, then applying to said exposed surface a coating of Portland cement in thin plastic condition and thereby causing the gelatinous substances in the coating in their initial process of formation, to chemically combine with the partially hardened gelatinous substances of the concrete.

4. The method of constructing upright concrete walls, which consists in providing mold forms spaced apart, in upright position, placing supporting devices in said space, pouring Portland cement concrete between the mold forms and permitting it to set and harden, then moving one of the mold forms to position spaced apart from the concrete and supporting it in said position and causing said supporting devices to extend across the space between the concrete and the said form that has been moved, then pouring Portland cement concrete into said space and permitting the concrete to remain in said position until the gelatinous substances formed therein have become sufficiently hardened to serve as a binder to hold the particles of the concrete together in a mass which is easily broken or crumbled, but which will be thus supported by the previously formed concrete wall and the supporting devices, then removing one of the mold forms and supporting the concrete in upright position from the side of the concrete opposite from the exposed surface, then applying to said exposed surface a coating of Portland cement in thin plastic condition and thereby causing the gelatinous substances in the coating in their initial process of formation, to chemically combine with the partially hardened gelatinous substances of the concrete, then applying pressure to said coating while being applied to the concrete for causing a physical union of the coating and wall.

WILLIAM ALLEN JENNINGS.